

Feb. 2, 1932.

J. TRAQUAIR

1,843,465

## PAPER MANUFACTURE

Filed April 27, 1928



## UNITED STATES PATENT OFFICE

JOHN TRAQUAIR, OF CHILlicothe, OHIO, ASSIGNOR TO THE MEAD CORPORATION, OF DAYTON, OHIO, A CORPORATION OF OHIO

## PAPER MANUFACTURE

Application filed April 27, 1928. Serial No. 273,241.

This invention relates to the manufacture of paper and the like from cellulose-containing materials, and particularly to the preparation of pulp to be used in such manufacture.

One of the principal objects of the invention is to provide a method of treating fibrous materials to produce a superior pulp product which may be formed into a paper having strength, color and other characteristics superior to the corresponding characteristics in paper formed from the same fibrous materials in other previously known ways.

Another object of the invention is to provide a method of chlorinating and bleaching fibrous materials to produce a pulp product which may be formed into a superior paper having unusual strength, purity and color.

Still another object of this invention is to provide a method of chlorinating and bleaching fibrous materials, which is continuous in operation, which is highly effective and easily controlled, and which effects a saving in the time of treatment and in the consumption of chemicals.

Still another object of the invention is to provide apparatus for carrying out the above method.

Other objects and advantages of the invention will be apparent from the following description when taken in connection with the accompanying drawing and appended claims.

In the drawing, the single figure is a diagrammatic illustration of a preferred form of apparatus constructed for carrying out the method of this invention.

In the manufacture of pulp from fibrous materials, it is the universal practice to subject the fibrous material to a chemical treatment which loosens and removes to a more or less degree the lignins and other incrustants which hold the fibers bound together, so that the fibers may be separated, after which the separate fibers, or pulp stock, is ordinarily subjected to a bleaching action to increase the whiteness of the fibers to the desired degree—depending on the field of utilization of the finished pulp stock. Because of the limitations heretofore imposed on this bleaching

action, it has been necessary, under old methods of pulping, to sacrifice either quantity of yield (with reference to the total quantity of fibrous material utilized), or quality of finished pulp.

This has been especially true with respect to certain types of fibrous materials, such as straw, flax, fibrous grasses, and the like. In such materials an inordinately large proportion of the fibrous material must be destroyed during the preliminary defibering, if the hard fiber bundles or shives, for example, are to be sufficiently defibered to permit of securing a final pulp of satisfactory whiteness using the bleaching methods heretofore known. Also with respect to certain hard woods, such as oak, chestnut, gum veneer cores, etc., for further example, the same thing has been true, and even with drastic defibering treatments it has not been commercially feasible to secure a suitable pulp from such woods.

The present invention provides a method of treating fibrous materials which have been given a preliminary defibering treatment so as to more or less completely separate the fibers thereof, whereby desired quality of pulp is secured without undue sacrifice in quantity. Particularly is this true with materials such as straw, in which the preliminary cook as ordinarily used fails to completely defiber the shives, etc. In carrying out this method suitably defibered material is subjected to successive treatments to produce pulp of unusual and superior strength and color characteristics, these treatments being hereinafter termed "halogenation" treatments for purposes of description.

The more or less defibered material is first subjected to the action of a halogenating agent such as a chlorinating agent in a manner to prevent a temperature rise of the mass undergoing chlorination such as to deleteriously affect the strength of the fibers. This may be accomplished by diluting the fibrous stock to a low consistency. In such case the water in which the fibers are suspended apparently serves as a heat-absorbing medium to avoid an objectionable temperature rise with injury to fibers. The water also serves

to dilute the hydrochloric acid formed in the reaction, this additionally diminishing objectionable results. Very satisfactory results have been secured with consistencies below 5%. Such low consistencies at the same time provide a fluent mass that may be readily pumped or flowed through conduits or treating chambers. This first stage of the chlorination is preferably continuous, the dilute stock being subjected to chlorination as it passes through the apparatus. The amount of chlorinating agent utilized is continuously controlled, preferably in an amount insufficient for complete chlorination. As a result the more readily chlorinated material 15 first reacts with the chlorinating agent in a comparatively short time as the mass flows along. The amount of chlorinating agent is preferably controlled to be as much as will be readily taken up by the fibers in this short 20 treating period, while insuring substantially complete reaction. This initial reaction is rapid, and it has been ascertained that the reaction of about 85% of the chlorine required for complete chlorination of a given fibrous mass goes to substantial completion in about fifteen to twenty minutes. Generally the addition of about 65% to 95% of the chlorine needed for complete chlorination in 25 the first stage with a treating time of about half an hour gives very satisfactory results. Various halogenating agents may be used for this first stage, chlorine being preferred due to the ease of control, and effectiveness and 30 rapidity of the reaction. However, the use of ordinary bleach or other calcium compounds at this point is found objectionable due to the formation of insoluble calcium reaction compounds in the pulp which are not readily washed out in the subsequent alkali 35 washing treatments. The chlorine may be added at a controlled rate in the form of chlorine water. Or the chlorine water solution may be added to the water in which the 40 fibers are suspended to provide the desired consistency. Or chlorine gas may be introduced at a controlled rate directly into the fibrous stream which has previously been 45 made down to the desired low consistency.

50 After this initial halogenation, it is found that the fibers may be subjected to a strong or drastic halogenating reaction with chlorine gas or bromine at high density or consistency without objectionable results. There will be 55 no deleterious temperature rise or deleterious acid formation under such secondary conditions, and the strength of the fibers is maintained and other high quality characteristics are secured. After such first-stage treatment 60 the fibrous mass is washed preferably with an alkali treatment, and is then thickened and rendered permeable to gas, and is then subjected to the action of a gaseous halogenating agent, such as chlorine gas, whereby the 65 chlorination is completed. In this phase of

more drastic action, in which a high chlorine concentration is effective in the fibrous mass, the chlorine gas reacts with the more resistant ligneous matter with consequent resolution of the shives or other undefibered material. 70 During such reaction the ligneous, and other material in the shives, or the like, is apparently changed by the action of the chlorine gas into compounds which may be readily washed out with alkaline solutions, or the like; or 75 which, even if not thus capable of being washed out, are of such character as to color, etc., as to be subsequently unobjectionable and ineffective to lower the quality characteristics of the resulting pulp. Very satisfactory results are secured in this phase with consistencies of substantially 15% or higher. The fibrous stock at such high density is 80 preferably passed continuously through a chamber having an atmosphere of chlorine 85 gas, in such wise that the chlorine gas thoroughly permeates the mass of fibers and effects intimate contact therewith. In practice it is desirable to secure continuous treatment throughout the entire chlorinating process, 90 and for this the rate of travel through the chamber may be so controlled as to effect continuous treatment of the material resulting from the treatment in the first stage. Generally a treating period of fifteen to thirty 95 minutes in this second stage is satisfactory, although a longer period may be used. The chlorinated pulp resulting is then steeped in alkali to dissolve out the reaction products of the chlorination, and washed. This pulp 100 may then be additionally bleached with a small amount of hypochlorite to secure a high white. The alkali steeping, washing and 105 bleaching are preferably continuous whereby the entire process may be continuously carried 110 out with accurate control and a minimum of attention.

Referring to the drawing, a pump is indicated at 10 for pumping the defibered material or washed "brown stock" coming from the digesters and wash pans or other pulping equipment, (not shown), through the pipe 11 to the chlorinating apparatus. The fibrous material at this point is diluted to a 115 low consistency such that objectionable temperature rise in the initial chlorination is prevented. A controlled supply of chlorinating agent such as chlorine water or chlorine gas, is introduced into the stream of fibrous material by pipe 12, which has a control valve 13. The fibrous mass and chlorinating agent pass together into a mixer 14 which comprises a length of pipe having a spiral baffle 15 therein to create turbulence in the flowing stock stream to mix the chlorinating agent with the mass, and from the mixer pass into a chlorinating tank or chamber 16. 120

The chlorinating tank 16 is constructed of acid-proof material such as tile or concrete 125

and is divided into a plurality of connected chambers or compartments, represented in the drawing by two chambers 17 and 18 divided by a central partition 19 terminating short of the bottom of the tank. The mixed mass and chlorinating agent flow downwardly through the space 17 and beneath the lower end of the partition 19, and up through the space 18 to the overflow pipe 20. The tank 16 is constructed of a capacity to accommodate sufficient material to provide the desired reaction time, as the stock flows from the inlet to the outlet.

The overflow outlet 20 discharges into a conventional type of washing apparatus, shown diagrammatically as a worm-type drum washer. This comprises essentially an acid-proof perforated rotary drum or screen 23 having an interior ribbon conveyor or spiral 24 and spray pipes 25 for spraying wash water upon the stock. The stock feeds into the interior of one end of the rotary drum, and is carried continuously through, being washed by the sprays and discharged from the other end, a part of the water therein draining through the perforated drum into a receiving tank 26 so that the stock generally discharges from the washer at a consistency of about 10% to 12%. The short time of treatment in the chlorination chamber coupled with the fact that the free acid formed in the reaction is washed out immediately after chlorination further serves to prevent injury to the fibers. An additional spray pipe 27 is preferably provided to direct an alkaline solution upon the washed fibers to neutralize any acid or free chlorine remaining in the fibrous mass thus avoiding the necessity for further acid-proof apparatus, as well as assisting in dissolving out reaction products of the chlorination. If desired, an alkaline steeping in addition to the washing may be given at this point, this being found advantageous in the case of fibrous stock which is less defibered.

The discharge 28 from the worm washer feeds to a further thickening device where the stock is dewatered to a consistency of substantially 15% or higher, preferably 20% to 30%, to render the pulp readily permeable to gas. This is preferably a continuous centrifugal machine of the type shown in the patent to Laughlin, 1,655,426, dated January 10, 1928. This machine comprises an inner distributing rotor 30 having a spiral flange 31, the rotor being keyed to a shaft 32 driven by a motor 33, and a second rotor or perforated filtering screen 34 carried by a sleeve 35 rotatably mounted upon shaft 32 and also driven from motor 33 through suitable gearing at a speed which is preferably slightly less than the speed of the rotor 30. The outer screen is surrounded by a stationary annular trough 36 forming an enclosing casing. The discharge 27 continuously feeds

the stock into the space between the inner rotor and the outer filtering screen, where it is carried through the machine by the spiral flange 31 while being subjected to such centrifugal force as to cause a portion of the retained water in the pulp to pass through the filtering screen 34 into the trough 36, from where the filtrate is removed by a pipe 36'. Other well-known types of continuous thickeners may be used for this purpose, such as rotary vacuum filters or cylindrical thickeners with pressure rolls to regulate the water content of the stock.

The dewatered stock discharged from the centrifugal machine is fed by a chute 37 to a supply trough 38 from where it is scooped by an endless bucket elevator 39 and fed into a treating tower 40 constructed of acid and chlorine proof material, where the second stage of the chlorination treatment is effected. Preferably a chlorinating tower such as that described in the application of John Traquair and Francis G. Rawling, Serial No. 273,242, filed of even date herewith, is used. As shown diagrammatically herein, the elevator 39 discharges into a hopper 42 which feeds into a screw conveyor 43 having an opening 44 on the lower side thereof opposite the open upper end 45 of the tower 40. Stock feeds through the opening 44 into the upper end of the tower 40 as needed to maintain the tower full of stock, the surplus stock handled by the screw conveyor 43 being discharged at the end 46 and returned to the source of supply. The tower 40 is provided with an inlet 48 for a controlled supply of chlorine gas, and controlled outlets 49 and 50 for the discharge of gas. The gas discharging from the tower, which contains some free chlorine, is preferably passed to recovery apparatus, (not shown) such as a water absorption system where chlorine water is formed which may be used in the first-stage chlorination. Water or other slushing liquid is introduced adjacent the base of the tower at 51 to dilute and slush out the stock through the water-sealed bottom 52 of the tower into a trough 53, the stock passing from the upper end to the lower end of the tower by gravity in accordance with the rate at which it is slushed out at the bottom, thereby providing a continuous travel of dewatered stock through a controlled and maintained atmosphere of chlorine gas.

The stock may be fed from the trough 53 to a storage tank, or it may be passed directly to further treating apparatus. As shown, the stock discharges through a pipe 56 into a solvent tank 57. Here it is mixed with a controlled quantity of alkali, continuously supplied from a pipe 58. The tank 57 is constructed to effect a continuous and uniform treatment of the material passing therethrough, and to secure a thorough mixing of the fibers with the solvent alkali. For this

purpose, the tank is provided with a plurality of staggered baffles 59 which provide a circuitous flow of the material from the inlet 60 to the discharge 61 connected to the suction side of a pump 62. The first compartment of the tank 57 is preferably provided with suitable agitating mechanism such as a driven shaft 65 having a plurality of rotary stirring arms 66. The capacity of the tank 57 is such that the treated material is allowed to remain about half an hour therein, this giving sufficient time for the reaction products of the chlorination to be dissolved. Any suitable alkali may be used for this purpose, dilute cold solutions of caustic soda, sodium carbonate, or sodium sulphite giving very satisfactory results.

The pump 62 feeds the dilute stock through a pipe 70 to a continuous filter mechanism 71 which serves to wash and thicken the treated material. This filtering mechanism may be a conventional rotary vacuum filter, such as an Oliver filter. This comprises a perforated rotary screen 72 divided into compartments of definite suction areas. The screen dips into the stock confined within a tank 73. The stock from pipe 70 together with sufficient water to make down to a consistency of about 1% is discharged into tank 73, and suction within the compartments of the screen causes the fibrous material to accumulate on the surface of the screen as the water passes into the suction compartments. As the screen rotates carrying the filtered fibrous material above the liquid level within the tank, sprays of wash water or dilute alkali are directed upon the material from spray pipes 74. The dissolved reaction products of the chlorination and the excess alkaline liquor are thus washed out of the stock, while controlled suction draws liquor from the fibrous layer. As the filter continues to rotate, the material which has thus been washed and thickened arrives at an area which is not subject to suction, and at this point a flexible scraper member 75 scrapes the material from the filter into a chute 76 which discharges into the first tank 80 of a bleacher which is preferably of the continuous type. The alkaline liquor and wash water drawn by suction into the interior of the rotary screen 72 are discharged through a central pipe 77. A portion of this alkaline liquor may be supplied to the spray pipe 27 of the worm washer.

Any suitable construction of continuous bleacher may be used. As shown, three connected tanks 80, 81 and 82, each having a rotary shaft 83 with agitating arms 84, are provided. The tanks are arranged at successively lower elevations, and the bottom of a preceding tank is connected to the upper end of a succeeding tank by a pipe connection 85. Each connection 85 has its highest point located below the level of the stock in the preceding tank, whereby a head is effec-

tive to secure a flow through the pipe. The capacity of the tanks is such as to insure sufficient time for the completion of the final bleaching action during the time the material flows through the connected bleaching tanks. A suitable bleaching agent, such as bleach liquor, sodium hypochlorite, or chlorine water is continuously added by pipe 86. Due to the effective chlorinating action, the quantity of bleach required is very materially reduced, approximately 1% to 3% of bleach liquor on the dry weight of the pulp being sufficient to produce a pulp having a high white color. The bleached pulp continuously discharging from the last tank 82 through pipe 88 is forced by a pump 89 to a second rotary vacuum filter 90 similar to the filter 71 where the pulp is washed and thickened. The treated pulp is then discharged through chute 91 into a stock chest 92 where it is stored for further treatment or for use.

The following is a typical example of a chlorinating treatment carried out in accordance with this invention. For the first-stage chlorination, chlorine water containing approximately 80% to 90% of the chlorine required for complete chlorination of the pulp is used. The chlorine is added to the stock in the form of a solution in water containing approximately .2% to .4% chlorine, or is added directly as chlorine gas. In the former case the raw fibrous material is made down to a consistency of about 4% to 6%, the addition of the chlorine water bringing the consistency to about 1% to 4%. In the latter case the consistency of the material is made down initially to about 2% or even less. The rate of flow through the chlorination chamber is controlled to give a treating time of about half an hour. The stock is then given an alkaline treatment and washing, and after thickening to about 20% to 30% consistency is then fed to the chlorinating tower where it is subjected to the second-stage chlorination by passing through a maintained layer of chlorine gas for about fifteen to thirty minutes. Both stages of the chlorination are carried on at ordinary room temperatures. The chlorinated stock is then introduced into the alkali solvent tank with a sufficient quantity of cold .1% NaOH solution to render the mass distinctly alkaline, and is agitated and steeped therein for about half an hour. After washing and making down to about 5% consistency, the material is introduced into the bleacher with a quantity of bleach liquor sufficient to bring the consistency to about 4% to 5% and to provide about 3% bleach liquor on the dry weight of the pulp. The flow of stock through the bleacher is controlled to provide a treating time of about one hour or more. A preliminary high density bleach may be given, if desired, before the stock is diluted to about 4% to 5%. The bleached

pulp is then washed and thickened and dropped to a stock chest.

While the method herein described, and the form of apparatus for carrying this method into effect, constitute preferred embodiments of the invention, it is to be understood that the invention is not limited to this precise method and form of apparatus, and that changes may be made in either without departing from the scope of the invention which is defined in the appended claims.

What is claimed is:

1. The method in the pulping of fibrous material which has been treated to separate its fibers, or defibered; which comprises diluting the defibered material to low consistency, subjecting the diluted material to the action of a halogenating agent, the consistency of said diluted material being controlled to prevent during halogenation a temperature rise of said diluted mass sufficient to deleteriously affect the strength of the fibers, then raising the consistency of said halogenated material, and subjecting said material of higher consistency to the action of a halogenating agent.

2. The method in the pulping of fibrous material, which comprises diluting defibered material to a consistency of less than 5%, subjecting the diluted material to the action of a halogenating agent, the consistency of the diluted material being controlled to prevent during the halogenation a temperature rise of said diluted mass sufficient to deleteriously affect the strength of the fibers, then dewatering the material to a consistency of substantially 15% or higher, and subjecting said dewatered material to the action of a halogenating agent in high concentration.

3. The method in the pulping of fibrous material, which comprises diluting defibered material to low consistency, treating said diluted material with a halogen-containing solution, the consistency of said diluted material being controlled to prevent during the treatment a temperature rise of the mass sufficient to deleteriously affect the strength of the fibers, thickening said treated material to render it permeable to gas, and then treating said thickened material with a gaseous halogen.

4. The method in the pulping of fibrous material, which comprises diluting defibered material to low consistency, chlorinating said diluted material with chlorine water, the consistency of said material being controlled to prevent during the chlorination a temperature rise of said mass sufficient to deleteriously affect the strength of the fibers, raising the consistency of said chlorinated material to render it permeable to gas, and then chlorinating the thickened material with chlorine gas.

5. The method in the pulping of fibrous material, which comprises first treating

fibrous material with a halogenating agent and concomitantly limiting the temperature rise of the mass as a result of such treatment to prevent deleteriously affecting the strength of the fibers, washing and thickening the treated material, and then subjecting the washed and thickened material to a strong halogenating action with a halogenating agent.

6. The method in the pulping of fibrous material, which comprises first chlorinating fibrous material with an insufficient amount of chlorinating agent to effect complete chlorination and concomitantly limiting the temperature rise of the mass as a result of such chlorination to prevent deleteriously affecting the strength of the fibers, washing and thickening the chlorinated material, and then completing the chlorination of the washed and thickened material with chlorine gas.

7. The method in the pulping of fibrous material, which comprises first treating fibrous material with a halogenating agent and concomitantly limiting the temperature rise of the mass as a result of such treatment to prevent deleteriously affecting the strength of the fibers, washing and thickening the treated material, treating the washed and thickened material with a gaseous halogenating agent, and treating the resultant mass with an alkaline solvent to dissolve out the reaction products of the halogenation.

8. The method in the pulping of fibrous material, which comprises first chlorinating fibrous material with a chlorinating agent and concomitantly limiting the temperature rise of the mass as a result of such chlorination to prevent deleteriously affecting the strength of the fibers, rendering said chlorinated material alkaline and washing without substantial delay, raising the consistency of said washed material to render it permeable to gas, chlorinating the thickened material with a gaseous chlorinating agent in high concentration, and treating the resultant material with an alkaline solvent and washing.

9. The method in the pulping of fibrous material, which comprises first chlorinating fibrous material with a chlorinating agent and concomitantly limiting the temperature rise of the mass as a result of such chlorination to prevent deleteriously affecting the strength of the fibers, washing and then raising the consistency of said chlorinated and washed material to render it permeable to gas, chlorinating the thickened material with chlorine gas, treating the resultant material with alkali and washing, and then bleaching said treated material.

10. The method in the pulping of fibrous material, which comprises diluting fibrous material to a consistency of less than 5%, chlorinating the diluted material with chlorine water, the consistency of the mass be-

ing controlled to prevent during the chlorination a temperature rise of said mass sufficient to deleteriously affect the strength of the fibers, dewatering said chlorinated material to a consistency of substantially 15% or higher, and chlorinating said dewatered material with chlorine gas.

11. The method in the pulping of fibrous material, which comprises diluting defibered material to low consistency, feeding the diluted material in a continuously flowing stream, introducing a halogenating agent into said flowing stream whereby halogenation of the material takes place as the mass flows along, continuously raising the consistency of the treated material to render it permeable to gas, and continuously treating said material of higher consistency with a halogenating agent in high concentration.

12. The method in the pulping of fibrous material, which comprises diluting defibered material to low consistency, feeding the diluted material in a continuously flowing stream, introducing a chlorinating agent into said flowing stream whereby chlorination of the material takes place as the mass flows along, the consistency of said mass being controlled to prevent during the chlorination a temperature rise of said mass sufficient to deleteriously affect the strength of the fibers, continuously raising the consistency of the chlorinated material to render it permeable to gas, and continuously feeding said material of higher consistency through an atmosphere of chlorine gas.

13. The method in the pulping of fibrous material, which comprises first treating fibrous material with a halogenating agent and concomitantly limiting the temperature rise of the mass as a result of such treatment to prevent deleteriously affecting the strength of the fibers, treating the halogenated material with alkaline solvent and washing, thickening the washed material, treating the thickened material with a halogenating agent, and then treating the material with an alkaline solvent and washing.

14. The method in the pulping of fibrous material, which comprises diluting defibered material to low consistency, feeding the diluted material in a continuously flowing stream, introducing a halogenating agent into said flowing stream whereby halogenation of the material takes place as the mass flows along, continuously treating the resultant material with an alkaline solvent and washing, continuously thickening the washed material to render it permeable to gas, continuously treating the thickened material with a gaseous halogenating agent, and then treating the material continuously with an alkaline solvent and washing.

15. The method in the pulping of fibrous material, which comprises diluting incompletely digested fibrous material to low con-

sistency, feeding the diluted material in a continuously flowing stream, introducing a halogenating agent into the flowing stream whereby reaction of the halogenating agent with the fibrous material takes place as the mass flows along, thickening the halogenated material, treating the thickened material with an alkaline solvent and washing, and then bleaching the washed material.

16. The method in the pulping of fibrous material, which comprises diluting incompletely digested fibrous material to low consistency, feeding the diluted material in a continuously flowing stream, introducing a halogenating agent into the flowing stream whereby reaction of the halogenating agent with the fibrous material takes place as the mass flows along, thickening the halogenated material to render it permeable to gas, passing the thickened material by gravity through an atmosphere of chlorine gas, removing the treated material from the chlorine atmosphere, and then treating the removed material with an alkaline solvent and washing.

17. The method in the pulping of fibrous material, which comprises diluting incompletely digested fibrous material to low consistency, feeding the diluted material in a continuously flowing stream, introducing a halogenating agent into the flowing stream whereby reaction of the halogenating agent with the fibrous material takes place as the mass flows along, treating the resultant material with an alkaline solvent and washing, thickening the washed material to a consistency of substantially 15% or higher, passing the thickened material by gravity downwardly through a maintained column of chlorine gas, removing the treated material from the maintained column and then treating the removed material with an alkaline solvent.

In testimony whereof I hereto affix my signature.

JOHN TRAQUAIR